

# UNITED STATES PATENT OFFICE.

STEPHEN M. ALLEN, OF WOBURN, MASSACHUSETTS.

## IMPROVEMENT IN THE MANUFACTURE OF PAPER FROM WOOD.

Specification forming part of Letters Patent No. 38,020, dated March 31, 1863.

*To all whom it may concern:*

Be it known that I, STEPHEN M. ALLEN, of Woburn, county of Middlesex, State of Massachusetts, have invented a new and improved method of preparing paper-stock from woody fibers—such as cotton-wood, bass-wood, poplar, whitewood, cane, and other woody matter of like fibrous substances—by a combined chemical and mechanical process; and I hereby declare that the following is a full, clear, and exact description of my method or process.

Woody fiber or the fiber of trees, shrubs, &c., as distinguished from the fiber connected with the bark of plants or coverings of seed-plants, like flax, hemp, or cereals, &c., have many valuable uses aside from those usually applied. Among these is that of its application to the production of paper-stock. While the structure of the ultimate fiber is very much the same in solid woody fiber as that of the fiber attached to the bark of plants, the method of treating the same is very different. The fiber connected with the bark of plants is held together almost entirely by a glutinous substance soluble under proper circumstances in warm water and alkalies, so that when removed the fiber is easily separated and fibrillized. That of wood, on the other hand, while possessing the same or an analogous glutinous substance for a cementing purpose, the fibrils themselves are mechanically wrought together, so that if the glutinous matter be removed the fibers would still hold strongly together. Thus it will be seen that while the fibrils of flax and hemp of from one to two inches long can be separated after the gummy matter is removed, those of the fiber of bass-wood, whitewood, and the like cannot be so separated even after the glutinous matter has been removed. The peculiar interlacing of the fibrils of wood is partially shown in bird's-eye maple, where the innumerable curlings and twistings are quite perceptible to the naked eye. The circulating action or capillary movement of the juices in the flax or hemp and the wood-fibers is also different. In the former they are caused to pass through the tubes of the fibrils, while in the latter it is between and through the little cells formed by the fibrils in their interlacings that the sap circulates.

Two difficulties arise in making paper-pulp from either woody fiber or flax, hemp, or like

substances—viz., the separation of the fibrils and the extraction of the gums and glutinous matter that surrounds the fiber of either. If this glutinous matter be not removed, the fiber cannot be bleached except at such strength of chlorine and acids as nearly to destroy the fiber, while the separation of the fiber by the usual process of grinding the pulp would pulvize rather than fibrilize the filaments.

Having thus stated the difficulties that are encountered in making paper from wood, I shall now proceed to describe my process of making paper-pulp and paper from woody fiber.

I take bass-wood, cotton-wood, poplar, whitewood, willow, birch, white pine, and, in fact, nearly all the varieties of wood found in the United States, except bird's-eye maple and pitch-pine, and saw or cut them up to convenient lengths for splitting into pieces of the length ordinarily used for shingles. I then crush the same between rollers or otherwise in such a way as to preserve the integrity of the fiber in its longitudinal direction, and afterward place the woody fiber thus prepared in a retort or boiler and subject the same to a series of steepings and washings in warm water, with or without alkaline or acid solutions, at different temperatures of heat. The first steeping I effect at about 105° Fahrenheit, after which the fiber is rinsed or washed. The second at about 140°, after which it is again rinsed or washed. For the third steeping I raise the temperature to about 170°, after which the same is again rinsed or washed. The mass may then be boiled until properly prepared for bleaching and grinding. When bleached and ground the pulp may be mixed with some other fiber or used plain in the manufacture of paper.

From the above it will be seen that the main object I have in view is the preservation of the length of fiber in the wood when fibrillized, so that it may be long enough for any kind of paper. The effect of steeping crushed or cut woody fiber prepared as before described in warm water or alkalies at different temperatures is to dissolve the glutinous and resinous matter contained in the wood, and which is readily dissolved at different temperatures below the boiling-point, but which coagulates or crystallizes when boiled. Thus by alternately steeping and washing the obnoxious elements

are removed, so that the filaments of wood will fibrilize instead of pulverize, and thus make a soft fiber sufficiently strong and fine for paper, while it will bleach readily and grind well in an ordinary paper-mill.

Having thus described my invention, I claim—

The manufacture of paper-pulp or paper from wood by performing the operations of cutting the wood in suitable lengths, crushing it in such manner as to preserve the integrity of the fiber in its longitudinal direction, alter-

nating steeping and washing the same at increased temperatures, and finally boiling, grinding, and bleaching the same, the whole in succession, substantially as herein described.

In testimony whereof I have signed my name to this specification before two subscribing witnesses.

STEPHEN M. ALLEN.

Witnesses:

L. BURNETT,  
HIRAM WELLINGTON.